

## UNITED STATES PATENT OFFICE

DAVID FRANKLIN YOUNGBLOOD, OF SAN ANTONIO, TEXAS

## STEEL ALLOY

No Drawing.

Application filed May 10, 1929. Serial No. 362,147.

This invention relates to hard steel alloys and aims to provide a special, tool-resistant, heat-resistant and rust-resistant steel, especially adapted for jails, vaults and the like, to prevent breaks from jails or theft from vaults, by the use of ordinary tools.

Heretofore, it has been customary to make jail and vault bars, plates and the like, of special laminated material composed of hard and soft layers, welded or fused together, the hard layers being included to render the composite material tool-resistant and the soft layers to make it sufficiently ductile to resist blows and strains and to facilitate its fabrication. The usual bars of this character consist of approximately 20% hard steel and 80% soft steel. However, long experience has taught that if such material is made sufficiently ductile to withstand blows and strains, it will not resist saws, files, and drills. Neither will it resist heat and rust. This invention aims to produce a special high-grade, alloy steel that possesses all of these necessary qualities in a solid form, without lamination.

One example of the improved alloy steel that has the foregoing qualities, includes the following materials:

|                     | Per cent     |
|---------------------|--------------|
| 30 Carbon -----     | 1.60 to 1.70 |
| Manganese -----     | 6.50 to 7.50 |
| Silicon -----       | 0.60 to 0.70 |
| Chromium -----      | 1.00 to 1.50 |
| Nickel -----        | 1.90 to 2.50 |
| 35 Molybdenum ----- | 0.25 to 0.40 |

The carbon, manganese, silicon, chromium and molybdenum all contribute to hardness and toughness without making the metal too brittle and to the heat resisting property, while the nickel adds greatly to the strength and ductility. Further, the nickel and possibly the manganese and chromium all contribute to making it rust-resistant. The relatively high percentage of carbon avoids the necessity of using more manganese and a part of the carbon is held in solution by the molybdenum when the metal is in the molten state. The silicon offsets, to some extent, the brittleness contributed by the manganese.

It has been found that this improved alloy steel has adequate ductility to afford the necessary strength for bars and plates such as are used in jails and vaults. It will withstand heavy blows and strains and bend considerably without breaking. It cannot be easily filed, sawed or drilled with ordinary tools. Neither is the hardness destroyed by the application of heat. Moreover, it is practically rust-proof and will last almost indefinitely. Thus, the material answers all of the necessary requirements for jail cells, vaults and the like.

## What is claimed is:

1. A tool-resistant and heat-resistant alloy steel of the character described containing 1.60 to 1.70% carbon, 6.50 to 7.50% manganese, 1.00 to 1.50% chromium, 1.90 to 2.50% nickel and 0.25 to 0.40% molybdenum.
2. An alloy steel having the properties described and containing 1.60 to 1.70% carbon, 6.50 to 7.50% manganese, 0.60 to 0.70% silicon, 1.00 to 1.50% chromium, 1.90 to 2.50% nickel and 0.25 to 0.40% molybdenum.

In testimony, that I claim the foregoing as my own, I have hereto affixed my signature.

DAVID FRANKLIN YOUNGBLOOD.